

Feb. 19, 1935.

C. R. E. WOHRMAN

1,991,438

THERMOSTATIC METAL

Filed Dec. 9, 1931



Carl R. E. Wohrman,  
Inventor,  
Delor F. Haynes  
Attorney

## UNITED STATES PATENT OFFICE

1,991,438

## THERMOSTATIC METAL

Carl R. E. Wohrman, Attleboro, Mass., assignor  
to General Plate Company, Attleboro, Mass., a  
corporation of Massachusetts

Application December 9, 1931, Serial No. 579,922

7 Claims. (Cl. 297—15)

This invention relates to thermostatic metal, and with regard to certain more specific features, to thermostatic metal particularly adapted for use under corrosive conditions, and/or at high 5 temperatures.

Among the several objects of the invention may be noted the provision of thermostatic metal of the class indicated which is capable of successfully withstanding the attack of corrosive 10 agencies, both liquid and gaseous, especially at intermediate temperatures (300—900° F.) and high temperatures (900° F. upwards); the provision of thermostatic metal of the class described which is capable of successful operation at temperatures 15 in excess of 1000° F.; and the provision of thermostatic metal of the class described which is readily formed from inexpensive, readily available material. Other objects will be in part obvious and in part pointed out hereinafter.

20 The invention accordingly comprises the elements and combinations of elements, features of construction and composition, and arrangements of parts, which will be exemplified in the structures and products hereinafter described; and the scope of the application of which will be indicated 25 in the following claims.

The accompanying drawing is a graph illustrating the temperature-expansion characteristics of certain alloys.

30 While a great variety of thermostatic metals have been and now are in use in temperature controlled devices, up to the present time none of the metals have been capable of successfully withstanding the attack of corrosive agencies generally. Attempts have been made to protect thermostatic metal elements by electroplating them, or otherwise plating them, with brass or a similar 35 corrosion-resistant medium. However, the porosity of such plating is objectionable; also, the fact that each element must be individually plated and polished makes such procedures quite impracticable. Welded or soldered plating ordinarily leaves the edges of the element unprotected, and even if the edges are protected, piercing of 40 the element as for mounting exposes the region around the piercing to attack. Further, platings of the above characteristics prove a deterrent to proper functioning of the element, and objectionably decrease its sensitivity.

45 Further, there has been up to the present time no thermostatic metal which operates successfully and consistently at temperatures in excess of 1000° F., retaining its elasticity at such temperatures and being at the same time free from destructive oxidation and scaling.

50 The present invention provides thermostatic metal which is adapted for use at the high temperatures in question, and which also successfully withstands the attack of such corrosive agencies,

thereby overcoming both of the above disadvantages.

While the present invention will be described in connection with the more usual thermostatic bimetal, comprising a composite sheet having two layers, each layer having a different temperature coefficient of expansion, it is to be understood that the invention is likewise applicable to trimetals, or any multimetal or like forms.

Proceeding with the description of the present 10 invention as applied more particularly to thermostatic bimetal, the individual metal layers will be considered.

The high expansion metal layer according to the present invention comprises a nickel-chromium steel of the stainless or heat-resisting variety. The range of composition of such nickel-chromium steel is approximately as follows:

|    | Per cent   |    |
|----|------------|----|
| Ni | 7-40       | 20 |
| Cr | 14-40      |    |
| C  | 0-3        |    |
| Mn | 0-3        |    |
| W  | 0-15       |    |
| P  | below 0.05 | 25 |
| S  | below 0.05 |    |
| Fe | balance    |    |

Phosphorus and sulphur are unavoidably present in small amounts as impurities. Molybdenum, silicon, cobalt, and vanadium may be added in amounts up to the order of 10% of each to improve the quality of the metal for special instances.

Nickel-chromium steels of the class indicated 35 are characterized by their high resistance to corrosion at ordinary as well as at elevated temperatures. This property permits the use of a thermostatic metal made from such nickel-chromium steels in corrosive media such as ammonia, sulphur-bearing fumes, acid and alkaline liquors, corrosive waters and oils, and sundry organic liquors and gases and the like. These nickel-chromium steels have at the same time an abnormally high resistance to oxidation and scaling 45 at high temperatures.

Nickel-chromium steels of the class described have a temperature coefficient of expansion of about  $16 \times 10^{-6}$  per degree C. for the temperature interval 0 to 200° C., and of about  $20 \times 10^{-6}$  50 for the temperature interval 0 to 1000° C. (See shaded area A of the drawing). Thus the coefficient of thermal expansion of such steels compares favorably with that of the Monel metal now extensively used in thermostatic metals in 55 the intermediate temperature field.

These nickel-chromium steels are adapted particularly for use as the higher expansion member of the thermostatic metal, the particular analysis (and heat treatment) being varied for 60

specific applications within the approximate limits indicated. As a non-limiting example, one suitable composition for use with low and intermediate temperature thermostatic metals is as follows:

|       | Per cent   |
|-------|------------|
| Ni    | 8-9        |
| Cr    | 18-19      |
| Mn    | 0.6        |
| 10 Si | 0.5        |
| W     | 0.1        |
| Mo    | 3          |
| C     | below 0.05 |
| S     | below 0.04 |
| 15 P  | below 0.04 |
| Fe    | balance    |

Another non-limiting example, being a suitable composition for high temperature (900° to 1500°) thermostatic metal is as follows:

|      | Per cent   |
|------|------------|
| Ni   | 25         |
| Cr   | 17½        |
| Mn   | 0.6        |
| Si   | 3          |
| 25 W | .15        |
| C    | below 0.15 |
| S    | below 0.04 |
| P    | below 0.04 |
| Fe   | balance    |

The nickel-chromium steels above described may be used with any suitable lower expansion member or members. For high temperature use, the stainless chromium irons hereinafter described are recommended. For low and intermediate temperatures, the currently employed nickel irons of the invar group containing some 36% to 48% nickel may be used, and, if necessary, protected by a coating of nickel chromium steel or some other metal or alloy resistant to the type of corrosion in question.

It will be understood that in many cases only one side of a thermostatic metal need be corrosion resistant, as in installations where the thermostat is mounted in the walls of the vessel and only one face is exposed to the corrosive medium. In such instances, the nickel-chromium steels described are desirable as the component metal coming in contact with the corrosive media, and it will be seen that any other suitable metal may be used as the other component of the thermostatic metal, it not being necessary for it to have, under such conditions, the quality of resisting corrosion.

55 The recommended metal for use as the lower expansion component in a high temperature thermostat hereinbefore indicated as chromium iron, comprises an alloy of that general description containing in excess of 14% chromium.

60 The range of composition of such chromium irons is substantially as follows:

|       | Per cent   |
|-------|------------|
| Cr    | 14-30      |
| Mn    | 0.3-0.7    |
| C     | 0-2.5      |
| W     | 0-15       |
| P     | below 0.05 |
| S     | below 0.05 |
| 70 Fe | balance    |

75 Molybdenum, silicon, cobalt, vanadium, and copper, in amounts up to about 10% each, may be added to improve the metal for specific applications. As a non-limiting example, adapted particularly for use with the first nickel-chromi-

um steel described, a suitable composition is as follows:

|    | Per cent   |
|----|------------|
| Cr | 17         |
| Mn | 0.3        |
| Si | 0.3        |
| C  | 0.06       |
| P  | below 0.04 |
| S  | below 0.04 |
| Fe | balance 10 |

Another non-limiting example, adapted particularly for use with the second nickel-chromium steel described, is as follows:

|    | Per cent   |
|----|------------|
| Cr | 20         |
| Mn | 0.3        |
| Si | 0.3        |
| C  | 0.07       |
| W  | 0.06       |
| P  | below 0.04 |
| S  | below 0.04 |
| Fe | balance    |

Chromium irons of the class indicated are characterized by their resistance to corrosion by a great variety of corrosive agencies at ordinary as well as at elevated temperatures and are able to stand occasional temperatures up to 1100° C. without defective oxidation or scaling. The chromium content is varied in accordance with the maximum temperature of which it is desired to use. A higher chromium content endows the alloy with a higher resistivity to corrosion at high temperatures. Conversely, a lower chromium content is sufficient in alloys which are to be used at lower temperatures.

Because the temperature coefficient of expansion of chromium irons of the class described is about  $10 \times 10^{-6}$  for the interval 0-200° C. and about  $12 \times 10^{-6}$  for the temperature interval 0-1000° C. (See shaded area B of the drawing.) It will be seen that this coefficient is considerably lower than that of the nickel chromium steel hereinbefore described, and it is thus a suitable metal to plate with the nickel chromium steel to form a thermostatic bimetal.

This temperature coefficient of expansion, however, is considerably higher than the temperature coefficient of expansion of invar or 42% nickel steel now extensively used, in the low and intermediate temperature fields, but is, however, lower than the coefficient of these metals at temperatures above the order of 350° C. Line C of the drawing represents a typical 42% nickel steel. Chromium irons, accordingly, are preferable even to the invar or 42% nickel steel for thermostatic metals operating at 350° C. or higher, even when the highly desirable corrosion resistivity characteristic is left out of consideration.

The higher expansivity of the chromium irons for temperatures up to 350° C. has the advantage of preventing the building up of unnecessary stresses in elements intended for use at, say, 500° C. and higher. In addition, there is sufficient deflection at lower temperatures to make the metal useful in elements adapted for such lower temperatures, especially in thermostats of a developable character in which small deflections and stresses are desired in order to prolong the life of the element.

While the chromium irons above described are used primarily as the lower expansion member in conjunction with the nickel chromium steels hereinbefore described, they are likewise adapted for advantageous use with other high expansion

members, such as Monel metal, nichrome, and the like.

Recapitulating, it will be seen that the present invention provides separate, new higher and lower expansion metals. These two metals are well adapted for use together, under the particular conditions described, but are each separately capable of use with known lower or higher expansion members as the case may be, to considerable advantage.

In view of the above, it will be seen that the several objects of the invention are achieved and other advantageous results attained.

As many changes could be made in carrying out the above constructions and compositions without departing from the scope of the invention, it is intended that all matter contained in the above description shall be interpreted as illustrative and not in a limiting sense.

20 I claim:

1. Thermostatic metal comprising a plurality of layers, the higher expansion of said layers having a composition substantially as follows:

|       | Per cent   |
|-------|------------|
| 25 Ni | 8-9        |
| Cr    | 18-19      |
| Mn    | 0.6        |
| Si    | 0.5        |
| W     | 0.1        |
| 30 Mo | 3          |
| C     | below 0.05 |
| S     | below 0.04 |
| P     | below 0.04 |
| 35 Fe | balance    |

and the lower expansion of said layers having a composition substantially as follows:

|       | Per cent   |
|-------|------------|
| 40 Cr | 17         |
| Mn    | 0.3        |
| Si    | 0.3        |
| C     | 0.06       |
| P     | below 0.04 |
| S     | below 0.04 |
| 45 Fe | balance    |

2. Thermostatic metal comprising a plurality of layers, the higher expansion of said layers having a composition substantially as follows:

|       | Per cent   |
|-------|------------|
| 50 Ni | 25         |
| Cr    | 17½        |
| Mn    | 0.6        |
| 55 Si | 3          |
| W     | 0.15       |
| C     | below 0.15 |
| S     | below 0.04 |
| P     | below 0.04 |
| 60 Fe | balance    |

and the lower expansion of said layers having a composition substantially as follows:

|       | Per cent   |
|-------|------------|
| 65 Cr | 20         |
| Mn    | 0.3        |
| Si    | 0.3        |
| C     | 0.07       |
| W     | 0.06       |
| P     | below 0.04 |
| 70 S  | below 0.04 |
| Fe    | balance    |

3. Thermostatic metal comprising a plurality of layers, the higher coefficient of expansion layer having a composition substantially as follows:

|    | Per cent |
|----|----------|
| Ni | 8-9      |
| Cr | 18-19    |
| Fe | balance  |

and the lower coefficient of expansion layer having a composition substantially as follows:

|    | Per cent |
|----|----------|
| Cr | 17       |
| Fe | balance  |

4. Thermostatic metal comprising a plurality of layers, the higher coefficient of expansion layer having a composition substantially as follows:

|    | Per cent |
|----|----------|
| Ni | 7-40     |
| Cr | 14-40    |
| Fe | balance  |

and the lower coefficient of expansion layer having a composition substantially as follows:

|    | Per cent |
|----|----------|
| Cr | 14-30    |
| Fe | balance  |

5. Thermostatic metal as set forth in claim 4, in which the composition of the higher coefficient of expansion layer is substantially as follows:

|    | Per cent   |
|----|------------|
| Ni | 8-9        |
| Cr | 18-19      |
| Mn | 0.6        |
| Si | 0.5        |
| W  | 0.1        |
| Mo | 3          |
| C  | below 0.05 |
| S  | below 0.04 |
| P  | below 0.04 |
| Fe | balance    |

6. Thermostatic metal as set forth in claim 4, in which the composition of the higher coefficient of expansion layer is substantially as follows:

|    | Per cent   |
|----|------------|
| Ni | 25         |
| Cr | 17½        |
| Mn | 0.6        |
| Si | 3          |
| W  | 0.15       |
| C  | below 0.15 |
| S  | below 0.14 |
| P  | below 0.04 |
| Fe | balance    |

7. Thermostatic metal as set forth in claim 4, in which the composition of the lower coefficient of expansion layer is substantially as follows:

|    | Per cent   |
|----|------------|
| Cr | 17         |
| Mn | 0.3        |
| Si | 0.3        |
| C  | 0.06       |
| W  | below 0.04 |
| P  | below 0.04 |
| S  | balance    |

CARL R. E. WOHRMAN. 70